# EUROPEAN PATENT SPECIFICATION

(11) **EP 3 470 542 B1**
(45) Date of publication and mention of the grant of the patent: **01.11.2023**
(21) Application number: 18196212.7
(22) Date of filing: 24.09.2018
(51) Int. Cl.: C22C 38/58, C22C 38/56, C22C 38/34, C22C 38/00, C22C 27/06, C22C 33/02

(54) **COBALT-FREE ALLOYS**
KOBALTFREIE LEGIERUNGEN
ALLIAGES EXEMPTS DE COBALT

(30) Priority: 11.10.2017 GB 201716640
(43) Date of publication of application: 17.04.2019
(73) Proprietor: Rolls-Royce plc, London N1 9FX (GB)
(72) Inventor: Stewart, David, Derby, Derbyshire DE24 8BJ (GB)
(74) Representative: Rolls-Royce plc

(56) References cited:
- WO-A1-02/02830
- GB-A- 1 459 255
- GB-A- 1 595 755
- JP-A- H11 226 778
- US-A- 2 799 577
- US-A- 4 494 988
- US-A- 4 814 140
- US-A1- 2015 368 766

## Description

### TECHNICAL FIELD

This disclosure relates to cobalt-free alloys.

### BACKGROUND

Cobalt-base alloys such as the Stellites (RTM) have been used extensively to form components or to provide hardfacing due to their high wear resistance, especially at high temperatures, with very good corrosion resistance. One application of such cobalt-base alloys is as a hardfacing on valve seats.

However, in a nuclear power plant, the use of cobalt-base alloys give rise to the potential for cobalt activation in the neutron flux which results in the radioisotope cobalt-60. The long half-life of cobalt-60 means that the use of cobalt-base alloys is generally undesirable in nuclear power plants.

United Kingdom Patent Number 1595755 discloses various alloys. One alloy, "Sample 3" in Table IV, has the following composition by weight-percentage: 0.070% carbon; 7.8% manganese; 4.2% silicon; 16.0% chromium; 6.0% nickel; 0.04% nitrogen; the balance being iron and incidental impurities.

Japanese Patent Application with publication number JP H11 226778 A discloses various alloys. Sample 42 has the following composition: 1.5% carbon; 4.0% silicon; 7.0% manganese; 34% chromium; 3.8% nickel; the balance being iron. Sample 43 has the following composition: 1.5% carbon; 4.0% silicon; 7.0% manganese; 30% chromium; 6.1% nickel; the balance being iron.

### SUMMARY

The invention is directed towards cobalt-free alloys. The alloy of the invention has an iron base and consists of, by weight:
0.8 to 2.5 percent carbon;
12 to 58 percent chromium;
7 to 9 percent manganese;
4 to 5 percent silicon;
4 to 6 percent nickel;
0.08 to 0.2 percent nitrogen;
the balance being iron plus incidental impurities.

The invention is defined in the appended claims.

### DETAILED DESCRIPTION

The alloy of the present invention has an iron base. The iron is, in the solid form of the alloy, in a predominantly austenitic crystallographic matrix. This is achieved by a depression of the martensite start temperature. By selecting a predominantly austenitic matrix, the formation of low-temperature phases which may occur in duplex matrixes is inhibited.

It will be appreciated that it is acceptable for there to be a quantity of other phases present in the solid form of the alloy in addition to the austenite. For example, it is acceptable for ferrite to be present, with no deleterious effects on performance. In a specific example, up to 8 percent of the iron may be in the form of ferrite.

The alloy further comprises carbon and chromium. As carbides precipitate on cooling, an appropriately-controlled cooling rate will allow the chromium to diffuse into chromium-depleted zones formed by the carbide precipitation. This is aided by the provision of a sufficient quantity of the chromium to, at meta-equilibrium, form a first population dissolved in the austenite for corrosion resistance, and a second population in the form of carbides. In one embodiment, the carbides may be either of the form Cr₇C₃. They may alternatively be in the form of Cr₂₃C₆. Alternatively there could be combination of those carbides. Other forms of chromium carbide may also be selectively formed.

The carbon is provided at an effective concentration of 0.8 to 2.5 percent by weight. The chromium is provided at a concentration of between 12 and 58 percent by weight. The lower bound of the chromium concentration is selected so as to ensure a sufficient quantity (a first population) is dissolved in the austenitic matrix for corrosion resistance. A second population of chromium combines with the carbon to form chromium carbides. The chromium carbides are provided at an effective concentration for galling resistance. They also provide general wear resistance.

In one embodiment, the first population of chromium is provided at a concentration of 16 percent by weight. The second population of chromium is provided at a concentration such that the molar ratio between chromium and carbon is 7:3. This allows the formation of Cr₇C₃. Alternatively, the second population of chromium is provided at a concentration such that the molar ratio between chromium and carbon is 23:6. This allows the formation of Cr₂₃C₆.

In one embodiment, the alloy has, by weight, 0.8 to 1.2 percent carbon. This produces an alloy which has comparable carbide content to Stellite 6. In another embodiment, the alloy has, by weight, 1.7 to 2.0 percent carbon. This produces an alloy which has comparable carbide content to Stellite 12. In another embodiment, the alloy has, by weight, 2.2 to 2.5 percent carbon. This produces an alloy which has comparable carbide content to Stellite 3.

It will be appreciated that chromium is a ferrite stabiliser, and indeed in high concentrations can completely eliminate the austenitic phase. This effect is offset however by provision of a sufficient concentration of austenite stabilisers to ensure the austenitic matrix is metastable at all temperatures that the alloy will be exposed to during service.

The austenite stabilisers maintain a predominantly austenitic crystallographic matrix in a metastable condition so as to prevent formation of ferrite during service. In this way, the quantity of dissolved chromium remains sufficient to maintain corrosion resistance.

The austenite stabilisers are nickel, manganese and nitrogen, with the overall concentration of these elements being selected so as to effect the required degree of austenite stabilisation.

The concentration of nickel required to depress the martensite start temperature sufficiently also increases the stacking fault energy of the austenitic matrix. The increase in stacking fault energy results in the matrix having a lower tolerance to defects introduced by deformation, such as galling. Thus, the nickel-equivalents manganese and nitrogen are also used so as to reduce the required nickel concentration.

Nitrogen also operates to reduce stacking fault energy throughout the entire austenitic matrix. This complements the carbide population in terms of providing resistance to galling.

It will be appreciated that chromium and manganese both increase the solubility of the nitrogen in the austenite, whilst having only a moderate propensity to form nitrides, and/or carbonitrides, compared with, for example, titanium which is a strong nitride former. In this way, higher concentrations of nitrogen may be used, thereby further reducing the amount of nickel required and further reducing stacking fault energy.

Furthermore, manganese not only acts as an austenite stabiliser and as a nitrogen solubility modifier, but it also acts to increase the hardenability of the alloy. Again, this acts to increase the galling resistance of the alloy.

Nickel also improves the corrosion resistance of the alloy over and above that achievable by provision of solely chromium for such a purpose. Manganese is abundant, as is nitrogen, thereby reducing difficulties in terms of sourcing supply of nickel.

The austenite stabilisers are provided in the following concentrations by weight: 7 to 9 percent manganese; 4 to 6 percent nickel; 0.08 to 0.2 percent nitrogen.

The carbide population is solely chromium-based. It has been found that whilst this may require measures to be taken to reduce sensitisation, it increases the corrosion resistance of the alloy relative to those embodiments where the additional carbide formers are provided.

In addition, it has been found that in gas atomisation production processes, the fast-quench from the melt does not give time for chromium carbides to form. Thus, the chromium and carbon content in the powder form of the alloy of the present invention remains in solution. The chromium carbides then precipitate during a HIP (hot isostatic pressing) process to produce or coat an article. Other carbides such as titanium carbide and vanadium carbide have been found to form and precipitate at higher temperatures, for example whilst the iron is still liquid, which in certain gas atomisation apparatus can cause nozzle blockages.

In order to facilitate production of a powdered form of the alloy, a melt fluidity promotor is included in the form of silicon at a concentration of 4 to 5 percent by weight. The powdered form of the alloy may be produced by gas atomisation.

It is envisaged that the alloys described herein may be provided in powdered form. Thus they may be used in, for example, a HIP process or a weld deposition process. The alloys may be used in a component part of a nuclear reactor. More generally, the alloys may constitute an article, or may constitute a coating of an article, for example a hardfacing. Additional heat treatments may be performed, for example to increase the quantity of austenite.

It will be understood that except where mutually exclusive, any of the features of the invention may be employed separately or in combination with any other features and the disclosure extends to and includes all combinations and sub-combinations of one or more features described herein.

## Claims

1. An alloy having an iron base, the alloy consisting of, by weight:
0.8 to 2.5 percent carbon;
12 to 58 percent chromium;
7 to 9 percent manganese;
4 to 5 percent silicon;
4 to 6 percent nickel;
0.08 to 0.2 percent nitrogen;
the balance being iron plus incidental impurities.

2. The alloy of claim 1, in which there is 16 percent by weight chromium forming a first population thereof, and a second population of chromium at a concentration such that the molar ratio between chromium and carbon is 7:3.

3. The alloy of claim 1, in which there is 16 percent by weight chromium forming a first population thereof, and a second population of chromium at a concentration a concentration such that the molar ratio between chromium and carbon is 23:6.

4. The alloy of any one of claims 1 to 3, in which there is, by weight: 0.8 to 1.2 percent carbon.

5. The alloy of any one of claims 1 to 3, in which there is, by weight: 1.7 to 2.0 percent carbon.

6. The alloy of any one of claims 1 to 3, in which there is, by weight: 2.2 to 2.5 percent carbon.

7. Powdered form of the alloy of any one of claims 1 to 6.

8. Use of the alloy of any one of claims 1 to 6 in a component part of a nuclear reactor.

9. An article comprising the alloy of any one of claims 1 to 6.

10. An article having a coating comprising the alloy of any one of claims 1 to 6.

## Patentansprüche

1. Legierung mit einer Eisenbasis, wobei die Legierung nach Gewicht aus Folgendem besteht:
0,8 bis 2,5 Prozent Kohlenstoff;
12 bis 58 Prozent Chrom;
7 bis 9 Prozent Mangan;
4 bis 5 Prozent Silizium;
4 bis 6 Prozent Nickel;
0,08 bis 0,2 Prozent Stickstoff;
wobei der Rest Eisen plus zufällige Verunreinigungen sind.

2. Legierung nach Anspruch 1, wobei es 16 Gewichtsprozent Chrom gibt, die eine erste Population davon bilden, und eine zweite Population von Chrom in einer Konzentration, sodass das Molverhältnis zwischen Chrom und Kohlenstoff 7:3 ist.

3. Legierung nach Anspruch 1, wobei es 16 Gewichtsprozent Chrom gibt, die eine erste Population davon bilden, und eine zweite Population von Chrom in einer Konzentration einer Konzentration, sodass das Molverhältnis zwischen Chrom und Kohlenstoff 23:6 ist.

4. Legierung nach einem der Ansprüche 1 bis 3, wobei es nach Gewicht Folgendes gibt: 0,8 bis 1,2 Prozent Kohlenstoff.

5. Legierung nach einem der Ansprüche 1 bis 3, wobei es nach Gewicht Folgendes gibt: 1,7 bis 2,0 Prozent Kohlenstoff.

6. Legierung nach einem der Ansprüche 1 bis 3, wobei es nach Gewicht Folgendes gibt: 2,2 bis 2,5 Prozent Kohlenstoff.

7. Pulverförmige Form der Legierung nach einem der Ansprüche 1 bis 6.

8. Verwendung der Legierung nach einem der Ansprüche 1 bis 6 in einem Komponententeil eines Kernreaktors.

9. Artikel, umfassend die Legierung nach einem der Ansprüche 1 bis 6.

10. Artikel mit einer Beschichtung, welche die Legierung nach einem der Ansprüche 1 bis 6 umfasst.

## Revendications

1. Alliage comportant une base de fer, l'alliage étant constitué par, en poids :
0,8 à 2,5 pour cent de carbone ;
12 à 58 pour cent de chrome ;
7 à 9 pour cent de manganèse ;
4 à 5 pour cent de silicium ;
4 à 6 pour cent de nickel ;
0,08 à 0,2 pour cent d'azote ;
le reste étant du fer plus des impuretés accidentelles.

2. Alliage selon la revendication 1, dans lequel sont présents 16 % en poids de chrome formant une première population de celui-ci, et une seconde population de chrome à une concentration telle que le rapport molaire entre le chrome et le carbone soit de 7:3.

3. Alliage selon la revendication 1, dans lequel sont présents 16 % en poids de chrome formant une première population de celui-ci, et une seconde population de chrome à une concentration une concentration telle que le rapport molaire entre le chrome et le carbone soit de 23:6.

4. Alliage selon l'une quelconque des revendications 1 à 3, dans lequel est présent, en poids :
0,8 à 1,2 pour cent de carbone.

5. Alliage selon l'une quelconque des revendications 1 à 3, dans lequel sont présents, en poids :
1,7 à 2,0 pour cent de carbone.

6. Alliage selon l'une quelconque des revendications 1 à 3, dans lequel sont présents, en poids :
2,2 à 2,5 pour cent de carbone.

7. Forme pulvérulente de l'alliage selon l'une quelconque des revendications 1 à 6.

8. Utilisation de l'alliage selon l'une quelconque des revendications 1 à 6 dans une pièce constitutive d'un réacteur nucléaire.

9. Article comprenant l'alliage selon l'une quelconque des revendications 1 à 6.

10. Article comportant un revêtement comprenant l'alliage selon l'une quelconque des revendications 1 à 6.
